# EUROPEAN PATENT SPECIFICATION

(11) **EP 2 468 903 B1**
(45) Date of publication and mention of the grant of the patent: **15.10.2014**
(21) Application number: 11195727.0
(22) Date of filing: 26.12.2011
(51) Int. Cl.: C21C 1/10, C22C 37/04, C22C 37/10

(54) **Manufacturing process of castings with spheroidal graphite**
Herstellungsverfahren von Gußstücken mit Kugelgraphit
Procédé de fabrication de moulages à graphite sphéroïdal

(30) Priority: 27.12.2010 ES 201031959
(43) Date of publication of application: 27.06.2012
(73) Proprietor: Frenos Iruña, S.A.L., 31191 Barbatain (Navarra) (ES)
(72) Inventor: Alvarez, Ignacio, 31191 Barbatain (Navarra) (ES)
(74) Representative: Pons Ariño, Angel

(56) References cited:
- EP-A1- 0 538 251
- AT-B- 344 765
- US-A1- 2008 296 098
- US-A1- 2009 191 085

## Description

The present invention relates to a process for the manufacturing of spheroidal castings by using metal or permanent molds. The resulting mechanical properties of the new parts are considered of great interest due to, among other things, the large number of graphite spheroids obtained in the parts.

### PRIOR STATE OF THE ART

The manufacturing of iron castings is mainly oriented to achieve economically competitive and metallic materials with suitable properties for the functionality of the components designed. In the latter case, part of current research efforts is directed towards obtaining graphite castings with optimized properties. The purpose of these "new cast materials" focuses on providing a more economical alternative to the use of steel or other special alloys for the manufacturing of high-performance parts.

Within the field of cast iron with precipitated graphite, spheroidal casting constitutes one of the materials that have been most widely used since its discovery in the 1950s. Compared to laminar or grey casting, the formation and subsequent growth of graphites in spheroidal form leads to significant increases in the break loads, the elastic limits, and, especially, in the elongations of the material. An adequate combination of these three mechanical properties entails the obtaining of materials with a wide range of technological applications.

The document AT344765 (WAAGNER BIRO AG, 1978) describes a procedure of obtainment of gray iron thick-walled castings, made of spherical graphite that comprises the use of "Kokillen" or metal inserts, which are situated in thermal centers, to increase the cooling velocity.

Moreover, the massive formation of graphite spheroids inside the metal matrix has even more interesting consequences. Under these conditions, the diffusion of carbon atoms [M. Wessén, I. Svensson, Metall. Mat. Trans. A, A27, 1996, 2209-2220] towards the numerous spheroids available during the cooling period of austenite (y-Fe) is favored. Consequently, suitable conditions are obtained for the formation and growth of ferrite (α-Fe) in the solid-solid transformation [J. Sertucha, R. Suárez, J. Izaya, L. A. Hurtado, J. Lagazpi, Int. J. Cast Met. Res., 2006, 19, 315-322]. This structural phase confers a high degree of ductility and impact resistance to the material, except in those cases wherein the contents of Si and/or P are high. [L. E. Björkegren, K. Hamberg, Proc. Keith Millis Symposium on Ductile Cast Iron, 2003*;* I. Riposan, M. Chisamera, S. Stan, Int J. Cast Met. Res, 20, 2007, 64-67]. On the other hand, the influence of cooling conditions on the structural characteristics and, consequently, the mechanical properties of cast iron with spheroidal graphite are well known [G. M. Goodrich, R. W. Lobenhofer, AFS Trans., 2007, 115, Working Paper No. 07-045, B. V. Kovacs, AFS Trans., 1981, 89, 79-96.]

The vast majority of current manufacturing processes use molds made with mixtures the primary component whereof is silica sand (Si02).

This refractory material is characterized by a comparatively low thermal conductivity, which greatly limits the cooling rate of the cast alloy inside this type of molds.

This type of technique has the following disadvantages:
- molding operations are more difficult, unmolding and the obtaining of parts is slow.
- presence of sand inclusions.
- low density of the spheroids per unit volume of material (less homogeneity in the properties of the material).
- due to the low solidification rate, greater additions of magnesium are required in the treatments in order to ensure a proper spheroidization index in the material.
- high risk of metal contraction.
- low yields in the molds (ratio between the metal in the parts and the metal cast in the mold).
- there is a possibility of deformation in the mold impressions due to the metallostatic pressure (lower dimensional precisions in the parts).
- need for subsequent finishing operations (burrs) in the parts.
- low thermal conductivity of the material and poor machinability.

For all these reasons, it is necessary to develop new methodologies for obtaining castings that improve the disadvantages outlined above.

### DESCRIPTION OF THE INVENTION

The present invention relates to a new process for the manufacturing of spheroidal cast iron parts, which solves all the disadvantages mentioned above, when molds made up of mixtures containing silica sand (SiO₂) as the primary constituent are used. This is done by using metal or "permanent" molds. The use of this new type of mold has the following advantages:
- Improved surface finish and minimal mold-metal interaction. Easier process for the surface cleaning of the parts.
- Ease of molding operations (it is only necessary to open and close the shells, in addition to the proper maintenance thereof).
- Speed in the unmolding and obtaining of the parts.
- Absence of sand inclusions (the most common defect in castings that use sand molds).
- High density of spheroids per unit volume of material (greater homogeneity in the properties of the material).
- Due to the increased solidification rate, it is necessary to add lower amounts of magnesium in the treatments in order to ensure a correct spheroidization index in the material.
- Low risk of metal contraction (minimization of shrink holes and microshrink holes).
- High yields in the molds (ratio between the metal in the parts and the metal cast in the mold).
- There is no possibility of deformations in the mold impressions caused by the metallostatic pressure (greater dimensional precision in the parts).
- If the molds are well-adjusted, subsequent finishing operations (burrs) on the parts are hardly necessary.
- Such a significant increase in the number of spheroids per unit volume results in an increase in the thermal conductivity of the material and improved machinability.

This new technique can be used for the manufacturing of castings for the automotive industry, hydraulic components, metal molds for the glass industry, centrifuged tubes, etc. The use of metal molds greatly accelerates the solidification rate and subsequent cooling of the material, causing major changes in the structures obtained in the as-cast state.

Therefore, a first aspect of the present invention is a process for manufacturing spheroidal castings, which comprises the following steps:
a) fusion of the metal loads at a temperature of between 1400 and 1600°C.
   More preferably, between 1430 and 1450°C.
b) adjustment of the metal loads to achieve the required composition;
c) spheroidization treatment at temperatures below 1148°C, and
d) casting process in metal or "permanent" molds.

According to a preferred embodiment, the metal loads are selected from the group formed by high carbon ingots, foundry chip briquettes, pig iron, scrap metal, steel from the automotive sector, returns or any combination thereof. Preferably, the metal loads are selected from high-carbon ingots, returns, foundry chip briquettes, steel from the automotive industry or any combination thereof.

According to another preferred embodiment, the composition of the metal loads is:
- between 25 and 90% of high-carbon ingots
- between 0 and 30% of steel from the automotive sector
- between 0 and 50% of foundry chip briquettes
- between 1 and 50% of returns

Always keeping in mind that the sum of all components must be 100%. Preferably, the composition of the metal loads is:
- between 30 and 80% of high-carbon ingots
- between 0 and 25% of steel from the automotive sector
- between 0% and 35% of foundry chip briquettes
- between 1 and 35% of returns

Always keeping in mind that the sum of all components must be 100%.

Even more preferably, the composition of the loads is:
- 75% of high-carbon ingots
- 20% of steel from the automotive sector
- 0% of foundry chip briquettes
- 5% of returns.
or
- 33.33% of high-carbon ingots
- 0% of steel from the automotive sector
- 33.33% of foundry chip briquettes
- 33.33% of returns

Always keeping in mind that the sum of all components must be 100%.

According to a preferred embodiment, after the adjustment of the metal loads the following composition is obtained:
- C: from 3.95 to 4.05% by weight.
- Si, from 1.00 to 2.60% by weight.
- Mn: from 0.40 to 0.80% by weight.
- S: from 0.00 to 0.20% by weight.
- Others:

More preferably, after the adjustment of the metal loads he following composition is obtained:
- C: from 3.60 to 4.05% by weight.
- Si, from 1.90 to 2.60% by weight.
- Mn: from 0.50 to 0.80% by weight.
- S: from 0.00 to 0.10% by weight.
- Others:

Always keeping in mind that the sum of all components must be 100%.

All these weight percentages are with respect to the total weight of the melt.

According to another preferred embodiment, the process of fusion of the metal loads is performed in rotary kilns. On the other hand, the melting and stay times of said metal load is 60 to 80 minutes (hours), preferably 70 minutes.

According to another preferred embodiment, in the step of adjusting the carbon and silicon contents, they are added depending on the content in the molten metal (metal loads) obtained in step a) in order to optimize the next step c) of spheroidization, such that the molten metal loads are transferred to at least 1 induction furnace (1000 Hz), preferably 3 induction furnaces. On the other hand, the temperature of the base metal is maintained within a range between 1400 and 1500°C, preferably between 1400 and 1450°C.

In another preferred embodiment, the spheroidization treatment comprises the following steps:
a. addition of FeSiMg in a proportion of 0.7 to 1.0% by weight with respect to the metal loads to be treated to the treatment ladle.
b. addition of an inoculant on the FeSiMg in a proportion of 0.15 to 0.20% by weight with respect to the metal loads to be treated.
c. addition of steel clippings so that these amply cover the FeSiMg and the inoculant previously entered into a reaction chamber;
d. filling of the metal loads from step b) to a 20 to 30% by volume of the ladle, guiding the fall of the metal towards the end opposite to a reaction chamber;
e. completing the filling of the ladle with the metal loads, and
f. slagging the metal treated.

According to a preferred embodiment, the FeSiMg alloy comprises the following composition:
- Si: from 30 to 60% by weight;
- Mg: from 1 to 30% by weight;
- Ca: from 0.1 to 4% by weight;
- Al: from 0.1 to 3% by weight;
- Rare earths: from 0 to 3% by weight, and
- Fe: from 30 to 60% by weight;

Even more preferably, the FeSiMg alloy comprises the following composition:
- Si: from 40 to 48% by weight;
- Mg: from 4 to 10% by weight;
- Ca: from 0.5 to 1.5% by weight;
- Al: from 0.3 to 1.2% by weight;
- Rare earths: from 0 to 1.3% by weight, and
- Fe: from 35 to 50% by weight;

According to another preferred embodiment, the inoculant comprises the following composition:
- Si: from 50 to 90% by weight;
- Ca: from 0.1 to 5.5% by weight;
- Al: from 0.1 to 5% by weight;
- Ba: from 0 to 15% by weight;
- Bi: from 0 to 5% by weight;
- Rare earths: from 0 to 4.5% by weight;
- Fe: from 15 to 35% by weight;

In an even more preferred embodiment, the inoculant comprises the following composition:
- Si: from 68 to 78% by weight;
- Ca: from 0.3 to 1.9% by weight;
- Al: from 0.3 to 1.5% by weight;
- Ba: from 0 to 9.5% by weight;
- Bi: from 0 to 1.2% by weight;
- Rare earths: from 0 to 1% by weight;
- Fe: from 20 to 30% by weight;

According to another preferred embodiment, stamped steel clippings are added until they cover the FeSiMg.

In another preferred embodiment, following the spheroidization step, a casting step is performed in metal or "permanent" molds. Said step comprises the following sub-steps:
a. transfer of the metal from the spheroidization step to a casting ladle equipped with an outlet siphon;
b. slagging of the treated metal from the previous step;
c. filling of the metal or permanent molds or through the siphon, ensuring that the ladle cup is full during the entire process of filling the molds;
d. vein addition (addition at the mold or shell inlet) of an inoculant to the casting metal in a weight percentage of 0.15% with respect to the metal treated in the ladle, the composition whereof is:
   - C: 3.70 to 3.85% by weight;
   - Si: 2.55 to 2.67% by weight;
   - Mn: 0.6 to 0.7% by weight;
   - P: 0.035 to 0.07% by weight;
   - S: 0.010 to 0.014% by weight;
   - Mg: 0.023 to 0.036% by weight, and
   - Cu: 0.01 to 0.02% by weight.
e. unmolding of the metal parts obtained, and
f. shot-blasting of the parts obtained in the previous step.

In the present invention, spheroidization is understood to mean a method for relieving the residual stresses in a high-carbon steel, consisting of heating for a long time at the lowest transformation temperature thereof, followed by slow cooling until it reaches room temperature.

Throughout the description and the claims, the word "comprise" and the variants thereof are not intended to exclude other technical characteristics, additives, components or steps. For persons skilled in the art, other objects, advantages and characteristics of the invention will become apparent partly through the description and partly through the practice of the invention. The following examples and drawings are provided by way of illustration and are not intended to limit the scope of the present invention.

### DESCRIPTION OF THE FIGURES

**Figure 1****.-** Figure 1 shows the configuration of the half-molds designed to manufacture jaws for the railway sector.
**Figure 2****.-** Heat treatment applied to the jaws in order to eliminate carbides.

The evolution of the temperature in one of the parts during application of the treatment.

### EXAMPLES

In the embodiment example, the implications arising from the use of silica sand or metal molds for the production of nodular castings with high requirements (wind energy sector) are comparatively studied. On the other hand, the advantages and disadvantages of using permanent molds in a production process are determined.

The fusion process of the materials was carried out in rotary kilns with a capacity of 5500 kg. The metal loads used were composed of 75% of high-carbon ingots, 20% of steel from the automotive sector and 5% of returns. Following the fusion of these loads, the resulting metal is transferred to three induction furnaces (1000 Hz) with a capacity of 1800 kg, in order to adjust the Carbon and Silicon contents (chemical composition by weight graphite: C ≥ 98%; FeSi: %Si = 74.6,%Al = 0.8, %Fe = 24.6) and raise the temperature of the base metal to 1400-1450°C. Table 1 shows the chemical composition ranges used in the preparation of the base metal.

**Table 1. Chemical compositions of the base metal**

| Element (%) | | | | | | |
|---|---|---|---|---|---|---|
| C | Si | Mn | P | S | Cu | Cr |
| 3.95-4.05 | 2.40-2.50 | 0.60-0.70 | 0.035-0.07 | 0.010-0.017 | 0.01-0.02 | 0.01-0.03 |

The spheroidization treatments of the base metal were made by transferring 70-75 kg from the electric furnaces to a ladle with a maximum capacity of 90 kg and equipped with a siphon outlet for the metal. Prior to carrying out this operation, the following were introduced, in this order, into the reaction chamber pertaining to this treatment ladle: 0.8% of the alloy FeSiMg621 (2-10 mm granulometry and chemical composition by weight: %Si = 44.1, %Mg = 6.8; %Ca = 2.2, %Al = 0.6, %RE = 1.2% and %Fe = 45.1), 0.15% of a commercial inoculant (0.5 to 3 mm granulometry and chemical composition by weight: %Si = 64.3; %Ca = 1.3,%Al = 0.9, %Ba = 9.3 and %Fe = 24.2) and stamped steel clippings as opacifying material. The discharge of metal from the electric furnace is performed such that the metal falls on the side opposite to that occupied by the reaction chamber at the bottom of the treatment ladle. The weight of the metal transferred was controlled with the aid of a dynamometer placed on the spoon.

After the treatment reaction with magnesium is completed, the slag was conveniently removed from the metal and the latter was quickly transferred to a ladle with a capacity of about 80 kg and equipped with an outlet siphon. The purpose of this device is to prevent the introduction of the slag formed inside the molds during the casting. The metal contained in the casting ladle was occasionally slagged off with this same aim. The casting of the molds was performed manually through the siphon, ensuring that the casting cup was kept full throughout the entire process of filling the molds. A post-inoculation of the casting metal was performed, by vein adding 0.15% of a commercial inoculant (0.2-0.7 mm granulometry and chemical composition by weight: %Si = 73.5; %Ca = 1.7, %Al = 1.0, %Bi = 0.9% and %Fe = 22.9).

**Table 2. Chemical compositions of the metal treated with Mg**

| Element (%) | | | | | | |
|---|---|---|---|---|---|---|
| C | Si | Mn | P | S | Cu | Cr |
| 3.95-4.05 | 2.40-2.50 | 0.60-0.70 | 0.035-0.07 | 0.010-0.017 | 0.01-0.02 | 0.01-0.03 |

The silica sand molds were manufactured using a high-pressure vertical molding line (12 kp/cm²) and mixtures composed of: 80.8% of re-used silica sand, 9.3% of activated sodium bentonite, 4.5% of carbonaceous material, 3.6% of water and 1.8% of new silica sand. The mixtures were sent to the molding machine with a compactibility of 38-41 %.

The permanent molds were manufactured by machining a crude foundry product, cast into a mold previously prepared for this purpose. The material used to prepare this crude product is flake graphite cast iron of the EN-GJL-200 grade.

After the machining and subsequent adjustment operations, the molds were coated internally with a layer of refractory paint and mounted on a carousel with a capacity for 12 molds, all equipped with an internal water refrigeration system. At each turn of the carousel, a system of acetylene-fed burners was used to provide a layer of coal dust on the refractory paint that covers the internal face of the metal molds. The addition of this carbonaceous layer may be regulated in each case. The temperature of the molds was controlled manually.

The parts used to conduct this study are: a component of the brakes used in wind furnaces and a clamping jaw for railway tracks. The weight of the brake caliper is 7.2 kg, showing sections between 5 and 43 mm. In the case of the jaw, the weight is 0.35 kg and sections vary between 5 and 12 mm. Thus, it is possible to evaluate the effect of different cooling rates in the same component. Figure 1 shows the configuration of the half-molds designed to manufacture jaws for use in the railway sector.

The parts manufactured in both the permanent molds and in those manufactured with the silica sand mixtures correspond to the brake caliper. The jaw was manufactured using only metal molds. After the manufacturing thereof, the parts were unmolded and, subsequently, shot blasted.

The materials of these parts were subjected to metallographic study in order to determine the spheroidization index (SI), the nodular density (N) and the composition of the metal matrix in different sections. The values of these parameters were obtained by analyzing 5 different observation fields in each sample and comparing them to standard patterns [15, 16]. On the other hand, the mechanical properties were determined on test-tubes machined directly on the parts. The dimensions of these test-tubes were dependent on the area of the part wherefrom they were obtained.

### RESULTS AND DISCUSSION

The structural characterizations were carried out in a narrow section and in a massive section, pertaining to three brake calipers manufactured in silica sand molds, three jaws and three brake calipers manufactured using metal molds, all of them as-cast. The results obtained from these studies are included in Table 3.

**Table 3. Results of the metallographic characterizations (as-casting parts), where SI represents the nodularity and N represents the no. of nodules per mm²**

| Brake calipers (metal mold) | | | | | | | | |
|---|---|---|---|---|---|---|---|---|
| Section (mm) | SI (%) | N (mm⁻²) | Nuclear structure (%) | | | Peripheral structure (%) | | |
| | | | Ferrite | Perlite | Carbides | Ferrite | Perlite | Carbides |
| 41 | >90 | 750-1100 | 85-100 | 15-0 | 0 | 90-100 | 10-0 | 0 |
| 8-9 | >90 | 950-1400 | 90-100 | 10-0 | 0 | 100 | 0 | 0 |

| Brake calipers (silica sand mold) | | | | | | | | |
|---|---|---|---|---|---|---|---|---|
| Section (mm) | SI (%) | N (mm-2) | Nuclear structure (%) | | | Peripheral structure (%) | | |
| | | | Ferrite | Perlite | Carbides | Ferrite | Perlite | Carbides |
| 41 | >90 | 180-220 | 30-35 | 70-65 | 0 | 15-25 | 85-75 | 0 |
| 8-9 | >90 | 340-480 | 10-20 | 90-80 | 0 | 2-10 | 98-90 | 0 |

| Jaws (metal mold) | | | | | | | | |
|---|---|---|---|---|---|---|---|---|
| Section (mm) | SI (%) | N (mm-2) | Nuclear structure (%) | | | Peripheral structure (%) | | |
| | | | Ferrite | Perlite | Carbides | Ferrite | Perlite | Carbides |
| 11 | >90 | 950-1400 | 35-40 | 65-60 | 0 | 20-30 | 80-68 | traces |
| 6 | >90 | 1300-1500 | 15-25 | 85-75 | 0-traces | 10-15 | 85-75 | 5-10 |

The comparative analysis of the data in Table 3 clearly shows the strong increase in the number of graphite spheroids when cooling of the material takes place inside the metal molds. This can be verified when comparing the brake calipers manufactured using silica sand molds to those obtained from the permanent molds. In the case of the clamping jaw, it is a smaller part and has narrower sections. However, for a similar cooling section, significant increases in the N parameter are not obtained as compared to the brake calipers. This reveals the strong influence of the solidification rate on the values of the N parameter obtained.

Another aspect to consider is the content of ferrite observed in each case. The calipers manufactured in the metal mold are largely or completely ferritic; however, those coming from the sand molds do not exceed 30-35% of this phase in any of the sections inspected (the content of manganese in the metal casting is 0.60 to 0.70%). This behavior must be primarily attributed to the presence of a greater number of graphite nodules per unit volume in the materials cooled in the metal mold. Thus, the distance between spheroids decreases considerably and the efficient diffusion of Carbon atoms from austenite is favored during the cooling thereof in the solid state, even though the latter is probably faster than in the parts manufactured inside the sand molds. It is necessary to consider that, when using permanent molds, the unmolding usually occurs 50-60 seconds after completing filling of the mold. In the case of manufactures with sand molds, this time may exceed 10 min.

When comparing the matrix structures in similar sections of the brake calipers and the jaws, both manufactured with metal molds, it is observed that the rate of cooling of austenite does exert an influence on the formation of ferrite during the eutectoid transformation. Even with higher values of the N parameter, the jaws show lower contents of this phase than the calipers (Table 3). This may be related to the size of the parts and the influence of this parameter on the cooling rate of the material when said parts are unmolded and remain in contact with air.

Another structural phase detected, which reveals the behavior described above, is iron carbides. This type of compounds are formed only in the clamping jaws, i.e. in the narrower sections with more critical cooling kinetics. It is logical to verify that the highest concentration of carbides was observed in the peripheral areas pertaining to the narrower sections in this part. The more rapid cooling that occurred in these areas in contact with the metal mold favors the appearance of carbide phases. In these cases, effective control of the temperature of the molds and ensuring effective inoculation in the metal casting becomes even more relevant.

The point is to add very active graphite nucleation elements (Ca, Si, Ba, Bi, etc.), which may counteract the effect exerted by the high solidification rate on the formation of carbides. In the process methodology used in this work two inoculations were performed: in the treatment with FeSiMg and a post-inoculation in the casting vein. However, it has not been possible to prevent the formation of carbides in the most critical sections of the jaws. The utility of the carbides formed in the peripheral areas as an effective measure to prevent wear in parts with specific applications has been suggested. In any case, proper inoculation of the metal casting also contributes to minimize the formation of contraction defects and increases the number of nodules, especially in the narrower sections, as has been demonstrated in the present work. Although we have not detected the presence of contraction defects, the literature includes publications dealing with the appearance of shrink holes and/or microshrink holes in parts manufactured in metal molds.

In order to eliminate the presence of carbides in the jaws, three other parts were selected and subjected to a standardized heat treatment. The temperature evolution in one of these parts during the application of this treatment is shown in Figure 2. The treated parts were metallographically inspected in order to confirm the total decomposition of the carbides and the presence of completely ferritic matrix structures in all the sections previously analyzed, which are specified in Table 3

With regards to the surface finish of the parts, after the unmolding and subsequent cooling to room temperature, those manufactured using permanent molds show a surface covered only by a thin dark layer of iron oxides. This layer can be easily removed with a short period of shot blasting. Comparatively speaking, the surface quality of the parts manufactured with metal molds is greater than that obtained with the sand molds. On the other hand, the dimensional precision obtained using metal molds is also greater and more repetitive.

The surface defects that may be observed in certain parts and most often are: slag and wrinkles or folds. In the first case, given the speed of the solidification period, it is very important to ensure the cleanliness of the metal casting and the effectiveness of the filling systems in preventing the entry of slag into the cavities that form the parts. With regard to surface wrinkles in spheroidal cast iron pieces, it was observed that they are favored when using longer casting times and/or, primarily, the temperatures of the metal molds are higher.

All the parts selected in this study were inspected by X-ray fluoroscopy in order to determine the presence of internal defects caused by contraction of the metal during the solidification stage. The metal molds prepared to manufacture both the brake caliper and the clamping jaw do not include any type of power system (Figure 1).

It is therefore necessary to evaluate the presence of shrink holes and/or microshrink holes in the manufactured parts for information on the behavior of the expansion-contraction balance of the metal in the interior of the metal molds. In no case was the presence of contraction defects detected in the selected parts manufactured in metal molds. The absence of this type of porosity must be related to the cooling kinetics applied when using this type of molds. By contrast, the brake calipers manufactured in sand molds do show microshrink holes with a variable size, mainly in the section changes close to the more massive sections of the part.

Table 4 shows the values of the maximum load at breakage (B), the elastic limit (EL) and the elongation (E) obtained from the traction assays performed to determine the mechanical properties of the selected parts. In the case of the clamping jaws, the mechanical assays were conducted only on the three parts subjected to the ferritization heat treatment described in Figure 2. In the brake calipers, all the materials were assayed in the as-cast state. The traction test-tubes were machined from two areas in each part. In the brake calipers, these areas correspond to the space designed for the hydraulic system (pot) and the central body (center). In the jaws, the test-tubes were obtained from the support wedge and the support area of the part.

**Table 4. Mechanical properties obtained on the part**

| As-cast brake calipers (metal mold) | | | | |
|---|---|---|---|---|
| Area | Test-tube diameter (mm) | B (MPa) | EL (MPa) | E (%) |
| Pot | 10 | 503-532 | 380-399 | 12-18 |
| Center | 10 | 505-520 | 376-402 | 13-20 |

| As-cast brake calipers (silica sand mold) | | | | |
|---|---|---|---|---|
| Area | Test-tube diameter (mm) | B (MPa) | EL (MPa) | E (%) |
| Pot | 10 | 605-710 | 367-418 | 9-11 |
| Center | 10 | 618-706 | 378-411 | 6-9 |

| Heat-treated jaws (metal mold) | | | | |
|---|---|---|---|---|
| Area | Test-tube diameter (mm) | B (MPa) | EL (MPa) | E (%) |
| Wedge | 5 | 435-466 | 294-313 | 18-20 |
| Support | 5 | 425-469 | 286-329 | 16-17 |

When comparing the mechanical properties of the brake calipers manufactured with metal and sand molds, the results obtained are consistent with the structural characteristics shown in Table 3. An increase in the solidification rate of the part inside the metal mold led to a strong increase in parameter N and a significant increase in the ferrite content.

These characteristics lead to materials that comfortably exceed 500 MPa of breakage load, with surprisingly high elastic limits (approximately 400 MPa) and elongations that may reach 20%. When transferring the part to molds manufactured with silica sand, materials are obtained with a greater load, a similar elastic limit and elongations that are clearly less than 12%.

In the case of the clamping jaw, the heat treatment applied transformed the structure, completely ferritizing it. Consequently, breakage loads are obtained that may exceed 450 MPa, elastic limits of about 300 MPa and elongations of up to 20%. Within this context, it must be borne in mind that they are results obtained directly on parts with a maximum section of 12 mm. Therefore, these results are of great interest, and they have a direct application in the design and subsequent manufacturing stages of nodular casting parts.

### CONCLUSIONS

The results obtained in the present work have shown that the use of metal molds is suitable for the manufacturing of spheroidal cast iron parts with significant functional requirements. The main structural implications resulting from the use of this type of molds are the significant increase in the number of graphite nodules per unit volume of material and a no less considerable increase in the ferrite content in the metal matrix obtained at room temperature.

Both structural characteristics make it possible to manufacture parts with interesting mechanical properties, especially the large elongations obtained in alloys with breakage loads greater than 510 MPa.

Therefore, the characteristics of the production process using metal molds and the results presented in this study should be taken into account when defining the most appropriate and cost-effective methodology for the production of spheroidal iron castings.

## Claims

1. Process for manufacturing spheroidal cast iron parts, which comprises the following steps:
a) fusion of the metal loads to a range of temperatures between 1400 and 1600°C; wherein the metal loads are selected from the group formed by high-carbon ingots, returns, foundry chip briquettes, steel from the automotive industry or any combination thereof;
b) adjustment of the carbon and silicon contents of the metal loads melted in step (a) to the following composition:
- C: from 3.95 to 4.05% by weight.
- Si: from 1.00 to 2.60% by weight.
- Mn: from 0.40 to 0.80% by weight.
c) spheroidization treatment of the metal loads obtained in step (b) at temperatures below 1148°C, comprising the following sub-steps:
a. addition of FeSiMg in a proportion of 0.7 to 1.0% by weight with respect to the total weight of the metal loads to a treatment ladle; wherein the alloy FeSiMg comprises the following composition up to 100%:
- Si: from 30 to 60% by weight;
- Mg: from 1 to 30% by weight;
- Ca: from 0.1 to 4% by weight;
- Al: from 0.1 to 3% by weight, and
- Fe: from 30 to 60% by weight.
b. addition of an inoculant on FeSiMg in a proportion of 0.15 to 0.20% with respect to the total weight of the metal loads; wherein the inoculant comprises the following composition up to 100%:
- Si: from 50 to 90% by weight;
- Ca: from 0.1 to 5.5% by weight;
- Al: from 0.1 to 5% by weight; and
- Fe: from 15 to 35% by weight.
c. addition of steel clippings to the mixture obtained in sub-step b.;
d. filling to 20 to 30% by volume of the ladle of the metal loads obtained in step b.;
e. addition of the molten metal loads from step b. until the ladle is filled, and
f. slagging off of the treated metal obtained in sub-step e,
and;
d) casting process of the metal loads obtained in step (c) in metal molds.

2. The method according to claim 1, wherein the metal load has the following composition up to 100%:
- between 25 and 90% of high-carbon ingots, preferably between 30 and 80%, and
- between 1 and 50% of returns, preferably between 1 and 35%.

3. The method according to claim 2, wherein the metal load further comprises:
- a percentage equal to or less than 30% of steel from the automotive sector, preferably a percentage equal to or less than 25%;
- a percentage equal to or less than 50% of foundry chip briquettes, preferably a percentage equal to or less than 35%;

4. The method according to claim 1, wherein the metal load has the following composition:
- 75% of high-carbon ingots;
- 20% of steel from the automotive industry, and
- 5% of returns.

5. The method according to claim 1, wherein the metal load has the following composition:
- 33.33% of high-carbon ingots;
- 33.33% of foundry chip briquettes, and
- 33.33% of returns.

6. The method according to any of claims 1 to 5, wherein the process of melting the metal loads is performed in rotary kilns, at a load fusion temperature between 1430 and 1450°C.

7. The method according to any of claims 1 to 6, wherein the fusing and stay times of said metal load is 60 to 80 minutes, preferably 70 minutes.

8. The method according to any of claims 1 to 7, where, in the step of adjusting the carbon and silicon content, the molten metal loads from step a) are transferred to at least 1 induction furnace, preferably 3 consecutive induction furnaces, and are maintained within a temperature range between 1400 and 1500°C, preferably at a temperature range between 1400 and 1450°C.

9. The method according to any of claims 1 to 8, wherein the alloy FeSiMg comprises the following composition up to 100%:
- Si: from 40 to 48% by weight;
- Mg: from 4 to 10% by weight;
- Ca: from 0.5 to 1.5% by weight;
- Al: from 0.3 to 1.2% by weight, and
- Fe: from 35 to 50% by weight.

10. The method according to claim 9, wherein the alloy FeSiMg further comprises a percentage equal to or less than 3% by weight of rare earths, preferably a percentage equal to or less than 1.3% by weight of rare earths.

11. The method according to any of claims 1 to 10, wherein the inoculant comprises the following composition up to 100%:
- Si: from 68 to 78% by weight;
- Ca: from 0.3 to 1.9% by weight;
- Al: from 0.3 to 1.5% by weight; and
- Fe: from 20 to 30% by weight.

12. The method according to claim 11, wherein the inoculant further comprises a percentage equal to or less than 15% by weight of Ba, a percentage equal to or 30 less than 5% by weight of Bi and a percentage equal to or less than 4.5% by weight of rare earths; preferably the inoculant comprises a percentage equal to or less than 9.5% by weight of Ba, a percentage equal to or less than 1.2% by weight of Bi and a percentage equal to or less than 1 % by weight of rare earths.

13. The method according to any one of claims 1 to 12, wherein step d), of casting in metal molds, comprises the following sub-steps:
a. transfer of the metal from the spheroidization step to a casting ladle equipped with an outlet siphon;
b. slagging off of the treated metal from the previous stage;
c. filling of the metal or permanent molds through a siphon;
d. vein addition of an inoculant to the metal casting, in a weight percentage of 0.15% with respect to the metal treated in the ladle, the composition whereof is:
- C: 3.70 to 3.85% by weight;
- Si: 2.55 to 2.67% by weight;
- Mn: 0.6 to 0.7% by weight;
- P: 0.035 to 0.07% by weight;
- S: 0.010 to 0.014% by weight;
- Mg: 0.023 to 0.036% by weight, and
- Cu: 0.01 to 0.02% by weight.
e. unmolding of the metal parts obtained, and
f. shot-blasting of the parts obtained in the previous step.

## Patentansprüche

1. Verfahren zur Herstellung von Gusseisenteilen mit Kugelgraphit, das folgende Schritte umfasst:
a) Aufschmelzen der Metallladungen auf eine Temperatur im Bereich von 1400 bis 1600 °C; wobei die Metallladungen ausgewählt werden aus der Gruppe bestehend aus kohlenstoffreichen Blöcken, Rückläufen, Gussspäne-Briketts, Stahl aus der Automobilindustrie oder jegliche Kombinationen davon;
b) Einstellen des Kohlenstoff- und des Siliciumgehalts der in Schritt (a) aufgeschmolzenen Metallladungen, um folgende Zusammensetzung zu erhalten:
- C: von 3,95 bis 4,05 Gew.-%
- Si: von 1,00 bis 2,60 Gew.-%
- Mn: von 0,4 bis 0,8 Gew.-%
c) Einformen der in Schritt (b) erhaltenen Metallladungen bei Temperaturen unter 1148 °C, das folgende Teilschritte umfasst:
a. Zugabe von FeSiMg in eine Behandlungsgießpfanne in einem Anteil von 0,7 bis 1,0 Gew.-% in Bezug auf das gesamte Gewicht der Metallladungen; wobei die FeSiMg-Legierung folgende Zusammensetzung zu 100 % umfasst:
- Si: von 30 bis 60 Gew.-%;
- Mg: von 1 bis 30 Gew.-%;
- Ca: von 0,1 bis 4 Gew.-%;
- Al: von 0,1 bis 3 Gew.-%; und
- Fe: von 30 bis 60 Gew.-%;
b. Zugabe eines Impfmittels zu FeSiMg in einem Anteil von 0,15 bis 0,20 % in Bezug auf das gesamte Gewicht der Metallladungen; wobei das Impfmittel folgende Zusammensetzung zu 100 % umfasst:
- Si: von 50 bis 90 Gew.-%;
- Ca: von 0,1 bis 5,5 Gew.-%;
- Al: von 0,1 bis 5 Gew.-%; und
- Fe: von 15 bis 35 Gew.-%;
c. Zugabe von Stahlschnitzeln zu der im Teilschritt b. erhaltenen Mischung;
d. Füllen der Gießpfanne bis zu 20 bis 30 Vol.-% mit der in Schritt b.
erhaltenen Metallladung;
e. Auffüllen der Gießpfanne mit der aufgeschmolzenen Metallladung aus Schritt b. und
f. Abschlacken des behandelten, im Teilschritt e. erhaltenen Metalls
und
d. Gießen der in Schritt (c) erhaltenen Metallladung in Metallgussformen.

2. Verfahren nach Anspruch 1, wobei die Metallladung folgende Zusammensetzung zu 100 % aufweist:
- 25 bis 90 % kohlenstoffreiche Blöcke, bevorzugt 30 bis 80 %, und
- 1 bis 50 % Rückläufe, bevorzugt 1 bis 35 %.

3. Verfahren nach Anspruch 2, wobei die Metallladung weiterhin Folgendes umfasst:
- einen Prozentsatz an Stahl aus dem Automobilsektor gleich oder unter 30 %, bevorzugt einen Prozentsatz gleich oder unter 25 %;
- einen Prozentsatz an Gussspäne-Briketts gleich oder unter 50 %, bevorzugt einen Prozentsatz gleich oder unter 35 %.

4. Verfahren nach Anspruch 1, wobei die Metallladung folgende Zusammensetzung aufweist:
- 75 % kohlenstoffreiche Blöcke;
- 20 % Stahl aus der Automobilindustrie und
- 5 % Rückläufe.

5. Verfahren nach Anspruch 1, wobei die Metallladung folgende Zusammensetzung aufweist:
- 33,33 % kohlenstoffreiche Blöcke;
- 33,33 % Gussspäne-Briketts und
- 33,33 % Rückläufe.

6. Verfahren nach einem der Ansprüche 1 bis 5, wobei das Verfahren des Aufschmelzens der Metallladungen in Drehrohröfen bei einer Schmelztemperatur der Ladung von 1430 bis 1450 °C durchgeführt wird.

7. Verfahren nach einem der Ansprüche 1 bis 6, wobei die Schmelz- und Standzeiten besagter Metallladung 60 bis 80 Minuten, bevorzugt 70 Minuten betragen.

8. Verfahren nach einem der Ansprüche 1 bis 7, wobei im Schritt des Einstellens des Kohlenstoff- und Siliciumgehalts die aufgeschmolzenen Metallladungen aus Schritt a) in mindestens einen Induktionsofen, bevorzugt in drei aufeinanderfolgende Induktionsöfen überführt werden und bei einer Temperatur im Bereich von 1400 bis 1500 °C, bevorzugt bei einer Temperatur im Bereich von 1400 bis 1450 °C gehalten werden.

9. Verfahren nach einem der Ansprüche 1 bis 8, wobei die FeSiMg-Legierung folgende Zusammensetzung zu 100 % umfasst:
- Si: von 40 bis 48 Gew.-%;
- Mg: von 4 bis 10 Gew.-%;
- Ca: von 0,5 bis 1,5 Gew.-%;
- Al: von 0,3 bis 1,2 Gew.-%; und
- Fe: von 35 bis 50 Gew.-%.

10. Verfahren nach Anspruch 9, wobei die FeSiMg-Legierung weiterhin einen Prozentsatz an Seltenen Erden gleich oder unter 3 Gew.-%, bevorzugt einen Prozentsatz an Seltenen Erden gleich oder unter 1,3 Gew.-% umfasst.

11. Verfahren nach einem der Ansprüche 1 bis 10, wobei das Impfmittel folgende Zusammensetzung zu 100 % umfasst:
- Si: von 68 bis 78 Gew.-%;
- Ca: von 0,3 bis 1,9 Gew.-%;
- Al: von 0,3 bis 1,5 Gew.-%; und
- Fe: von 20 bis 30 Gew.-%.

12. Verfahren nach Anspruch 11, wobei das Impfmittel weiterhin einen Prozentsatz an Ba gleich oder unter 15 Gew.-%, einen Prozentsatz an Bi gleich oder unter 5 Gew.-% und einen Prozentsatz an Seltenen Erden gleich oder unter 4,5 Gew.-% umfasst; wobei das Impfmittel bevorzugt einen Prozentsatz an Ba gleich oder unter 9,5 Gew.-%, einen Prozentsatz an Bi gleich oder unter 1,2 Gew.-% und einen Prozentsatz an Seltenen Erden gleich oder unter 1 Gew.-% umfasst.

13. Verfahren nach irgendeinem der Ansprüche 1 bis 12, wobei der Schritt d) des Gießens in Metallgussformen folgende Teilschritte umfasst:
a. Überführen des Metalls aus dem Schritt des Einformens in eine mit einem Ausgusssiphon ausgestattete Gießpfanne;
b. Abschlacken des behandelten Metalls aus der vorangegangenen Stufe;
c. Einfüllen des Metalls in Kokillen über einen Siphon;
d. Zugabe eines Impfmittels zum Metallguss in einem Gewichtsprozentsatz von 0,15 % in Bezug auf das in der Gießpfanne behandelte Metall, dessen Zusammensetzung folgende ist:
- C: 3,70 bis 3,85 Gew.-%;
- Si: 2,55 bis 2,67 Gew.-%;
- Mn: 0,6 bis 0,7 Gew.-%;
- P: 0,035 bis 0,07 Gew.-%;
- S: 0,010 bis 0,014 Gew.-%;
- Mg: 0,023 bis 0,036 Gew.-%; und
- Cu: 0,01 bis 0,02 Gew.-%;
e. Entformen der erhaltenen Metallteile und
f. Kugelstrahlen der im vorangegangenen Schritt erhaltenen Teile.

## Revendications

1. Procédé pour fabriquer des pièces sphéroïdales en fonte, qui comprend les étapes suivantes :
a) fusion des charges de métal à des températures comprises entre 1400°C et 1600°C ; dans lequel les charges de métal sont sélectionnées dans le groupe formé par des lingots à haute teneur en carbone, des retours, des briquettes de copeaux de fonderie, de l'acier provenant de l'industrie automobile ou n'importe laquelle de leurs combinaisons ;
b) ajustement des teneurs en carbone et silicium des charges de métal fondues durant l'étape (a) à la composition suivante :
- C : de 3.95 à 4.05% en poids ;
- Si : de 1.00 à 2.60% en poids ;
- Mn : de 0.4 à 0.8% en poids.
c) traitement de sphéroïdisation des charges de métal obtenues durant l'étape (b) à des températures inférieures à 1148°C, comprenant les sous-étapes suivantes :
a. ajout de FeSiMg dans une proportion de 0.7 à 1.0% en poids par rapport au poids total des charges de métal à une poche de traitement ; dans lequel l'alliage FeSiMg comprend la composition suivante jusqu'à 100% :
- Si : de 30 à 60% en poids ;
- Mg : de 1 à 30% en poids ;
- Ca : de 0.1 à 4% en poids ;
- Al : de 0.1 à 3% en poids, et
- Fe : de 30 à 60% en poids.
b. ajout d'un inoculant sur FeSiMg dans une proportion de 0.15 à 0.20% en poids par rapport au poids total des charges de métal ; dans lequel l'inoculant comprend la composition suivante jusqu'à 100% :
- Si : de 50 à 90% en poids ;
- Ca : de 0.1 à 5.5% en poids ;
- Al : de 0.1 à 5% en poids, et
- Fe : de 15 à 35% en poids.
c. ajout de rognures d'acier au mélange obtenu durant la sous-étape b. ;
d. remplissage de 20 à 30% en volume de la poche avec les charges de métal obtenues durant l'étape b. ;
e. ajout des charges de métal en fusion de l'étape b. jusqu'à ce que la poche soit remplie, et
f. décrassage du métal traité obtenu durant la sous-étape e, et
d. procédé de coulée des charges de métal obtenues durant l'étape (c) dans des moules en métal.

2. Le procédé selon la revendication 1, dans lequel la charge de métal a la composition suivante jusqu'à 100% :
- entre 25 et 90% de lingots à haute teneur en carbone, de préférence entre 30 et 80%, et
- entre 1 et 50% de retours, de préférence entre 1 et 35%.

3. Le procédé selon la revendication 2, dans lequel la charge de métal comprend en outre :
- un pourcentage égal ou inférieur à 30% d'acier provenant du secteur automobile, de préférence un pourcentage égal ou inférieur à 25% ;
- un pourcentage égal ou inférieur à 50% de briquettes de copeaux de fonderie, de préférence un pourcentage égal ou inférieur à 35% ;

4. Le procédé selon la revendication 1, dans lequel la charge de métal a la composition suivante :
- 75% de lingots à haute teneur en carbone ;
- 20% d'acier provenant de l'industrie automobile, et
- 5% de retours.

5. Le procédé selon la revendication 1, dans lequel la charge de métal a la composition suivante :
- 33.33% de lingots à haute teneur en carbone ;
- 33.33% de briquettes de copeaux de fonderie, et
- 33.33% de retours.

6. Le procédé selon n'importe laquelle des revendications 1 à 5, dans lequel le processus de fusion des charges de métal s'effectue dans des fours rotatifs, à une température de fusion de la charge entre 1430 et 1450°C.

7. Le procédé selon n'importe laquelle des revendications 1 à 6, dans lequel les temps de fusion et d'attente de ladite charge de métal est de 60 à 80 minutes, de préférence de 70 minutes.

8. Le procédé selon n'importe laquelle des revendications 1 à 7, où, durant l'étape d'ajustement de la teneur en carbone et silicium, les charges de métal en fusion de l'étape a) sont transférées dans au moins 1 four à induction, de préférence 3 fours à induction consécutifs, et sont maintenues à une température comprise entre 1400 et 1500°C, de préférence à une température entre 1400 et 1450°C.

9. Le procédé selon n'importe laquelle des revendications 1 à 8, dans lequel l'alliage FeSiMg comprend la composition suivante jusqu'à 100% :
- Si : de 40 à 48% en poids ;
- Mg : de 4 à 10% en poids ;
- Ca : de 0.5 à 1.5% en poids ;
- Al : de 0.3 à 1.2% en poids, et
- Fe : de 35 à 50% en poids.

10. Le procédé selon la revendication 9, dans lequel l'alliage FeSiMg comprend en outre un pourcentage égal ou inférieur à 3% en poids de terres rares, de préférence un pourcentage égal ou inférieur à 1.3% en poids de terres rares.

11. Le procédé selon n'importe laquelle des revendications 1 à 10, dans lequel l'inoculant comprend la composition suivante jusqu'à 100% :
- Si : de 68 à 78% en poids ;
- Ca : de 0.3 à 1.9% en poids ;
- Al : de 0.3 à 1.5% en poids, et
- Fe : de 20 à 30% en poids.

12. Le procédé selon la revendication 11, dans lequel l'inoculant comprend en outre un pourcentage égal ou inférieur à 15% en poids de Ba, un pourcentage égal ou inférieur à 5% en poids de Bi et un pourcentage égal ou inférieur à 4.5% en poids de terres rares, de préférence l'inoculant comprend un pourcentage égal ou inférieur à 9.5% en poids de Ba, un pourcentage égal ou inférieur à 1.2% en poids de Bi et un pourcentage égal ou inférieur à 1 % en poids de terres rares.

13. Le procédé selon n'importe laquelle des revendications 1 à 12, dans lequel l'étape d), de coulée dans des moules en métal, comprend les sous-étapes suivantes :
a. transfert du métal de l'étape sphéroïdisation dans une poche de coulée équipée d'un siphon d'évacuation ;
b. décrassage du métal traité de l'étape précédente ;
c. remplissage des moules de métal ou permanents via un siphon ;
d. ajout d'une veine d'un inoculant à la coulée de métal, dans un pourcentage de poids de 0.15% par rapport au métal traité dans la poche, dont la composition est :
- C : 3.70 à 3.85% en poids ;
- Si : 2.55 à 2.67% en poids ;
- Mn : 0.6 à 0.7% en poids :
- P : 0.035 à 0.07% en poids ;
- S : 0.010 à 0.014% en poids ;
- Mg : 0.023 à 0.036% en poids, et
- Cu : 0.01 à 0.02% en poids.
e. démoulage des pièces de métal obtenues, et
f. grenaillage des pièces obtenues durant l'étape précédente.
